

# UNITED STATES PATENT OFFICE.

REGINO A. MARTINEZ, OF BUENOS AIRES, ARGENTINA, ASSIGNOR TO PEDRO EUGENIO GIRARD, OF BUENOS AIRES, ARGENTINA.

## IGNITING SUBSTANCE.

1,338,389.

Specification of Letters Patent. Patented Apr. 27, 1920.

No Drawing.

Application filed June 30, 1919. Serial No. 307,851.

To all whom it may concern:

Be it known that I, REGINO ALEJANDRO MARTINEZ, a citizen of the Argentine Republic, residing at No. 452 Corrientes street, 5 Buenos Aires, Argentine Republic, have invented certain new and useful Improvements in Igniting Substances, of which the following is a specification.

The present invention refers to an igniting substance susceptible of being applied to a combustible body and has for its object an igniting paste intended to be applied directly to the body or substance which it is required to ignite.

15 The present invention has also for its object a composition which by means of friction permits of setting fire to the aforementioned paste.

The paste in accordance with the present 20 invention may be used in many ways, being specially applicable to cigars and cigarettes, thus dispensing with the use of matches.

The paste to which this invention refers 25 possesses, over all others proposed up to the present, the advantages of reduced cost, freedom from substances harmful to health, the fact that it produces neither noise nor flame on ignition, that it is not harmed by dampness, and finally, that it cannot ignite by 30 itself, it being necessary for the latter purpose to bring it into frictional contact with a special paste which is also comprised in the present invention.

The principal paste, designed to set fire to 35 the required body, is constituted by the following elements, substantially in the proportions specified:

|                         |     |
|-------------------------|-----|
| Chlorate of potassium   | 35% |
| Bichromate of potassium | 2%  |
| 40 Starch               | 40% |
| Sawdust                 | 10% |
| Tragacanth gum          | 3%  |
| Vegetable charcoal      | 10% |

45 This composition is weak and cannot be set alight by friction.

It is ignited by means of another sensitive composition or paste composed as fol-

lows and substantially in the proportions indicated:

|                         |     |
|-------------------------|-----|
| Chlorate of potassium   | 45% |
| Sulfid of antimony      | 30% |
| Gum arabic              | 8%  |
| Bichromate of potassium | 2%  |
| 55 Glass powder         | 10% |
| Bioxid of lead          | 5%  |

This paste ignites only on friction with a special paste which forms a rough surface and which may be applied to any independent body, and the composition of which is as follows:

|                         |     |
|-------------------------|-----|
| Amorphous phosphorus    | 30% |
| Sulfid of antimony      | 18% |
| 60 Glass powder         | 35% |
| Bichromate of potassium | 2%  |
| Glue                    | 15% |

It is evident that slight changes may be made in the composition of the several pastes 70 and that they may be applied to the body which it is required to ignite, in any suitable manner, without thereby departing from the scope of the invention, which is clearly determined in the claims which follow this 75 specification.

Having now specifically described and determined the nature of the present invention and the method of its employment, I declare that what I claim as my invention and exclusive right is:

1. A new industrial product consisting in an inflammable substance capable of being applied directly to the objects or bodies which are to be ignited, characterized by the 85 fact that it is constituted by an igniting paste applied directly to the required body and answering substantially to the formula:—chlorate of potassium 35%; bichromate of potassium 2%; starch 40%; sawdust 90 10%; tragacanth gum 3%; vegetable charcoal 10%.

2. A composition intended to permit of the ignition by friction of the inflammable paste, in accordance with claim 1, characterized by the fact that it answers substan- 95

5 tially to the formula:—amorphous phosphorus 30%; sulfid of antimony 18%; glass powder 35%; bichromate of potassium 2%; glue 15%, substantially as described and for the purposes specified.

3. A new industrial product consisting of an inflammable substance capable of being applied directly to the objects or bodies which are to be ignited, and a sensitive paste

superimposed upon the inflammable substance and answering substantially to the formula:—chlorate of potassium 45%; sulfid of antimony 30%; gum arabic 8%; bichromate of potassium 2%; glass powder 10%; bioxid of lead 5%, substantially as described and for the purpose specified.

In testimony whereof I affix my signature.

REGINO A. MARTINEZ.